

## UNITED STATES PATENT OFFICE

2,007,341

## PROCESS OF TREATING CELLULOSE FIBERS

Fredrich Olsen and Frederick R. Seavey, Dover,  
N. J., assignors to The Cellulose Research Corporation, a corporation of Delaware

No Drawing. Application February 13, 1929,  
Serial No. 339,732

7 Claims. (Cl. 92—1)

(Filed but not issued under the act of March 3,  
1883, as amended April 30, 1928; 370 O. G. 757)

The invention described herein may be manufactured and used by us for the Government for governmental purposes, without the payment to us of any royalty thereon.

5 This invention relates to a process of treating cellulose fibers.

In the preparation of nitrocellulose explosives, the cellulose is nitrated in a bath of nitric and sulphuric acid. When removed from the bath, 10 the tubular fibers carrying both adherent or mechanically-held acid and adsorbed acid as well as other impurities must be subjected to a purification treatment to remove these unstable lower nitro bodies.

15 The principal object of this invention is the reduction of the fibers to a physical condition which will be favorable for the action of the purifying or neutralizing agents. This object is attained by filling the tubular fiber with a substance capable, under given conditions, of rapidly changing its state and by reason of such change producing a pressure within the fiber sufficient to disrupt the same.

20 In the method of disrupting wood and other ligno-cellulose materials by an explosion process consisting of suddenly reducing the external pressure, the pressure fluid medium is capable of penetrating the material because of its rigidity. This condition does not obtain in cellulose reduced to a mass of single unsupported fibers 25 which because of their normal thin-walled tubular structure would be compressed or collapsed by the pressure fluid medium and, since the tube is not filled with the fluid, there can be no balancing of interior and exterior pressures preliminary to the reduction of external pressure.

30 It is, therefore, proposed to prepare the tubular fibers against collapse by filling them with a relatively incompressible fluid. This condition 35 of the fibers may be produced by allowing them to become saturated with a liquid, conveniently water, and also optionally by removing the entrapped air from the fibers by the application of a vacuum.

40 The fibers thus prepared are placed in a high pressure chamber and a fluid of high temperature such as steam is admitted to the chamber under a pressure of 500 to 1000 pounds per square 45 inch and for periods varying from five seconds

to one minute, depending upon the degree of physical disruption it is desired to secure. Upon suddenly relieving the pressure as by discharging the fibers through an opening in the chamber, the fluid in the fibers which has been heated by the pressure medium is rapidly converted into steam causing disruption of the fibers.

5 We claim:

1. The step in the preparation of smokeless powder which consists in filling each fiber of a 10 mass of collapsible cellulose fibers with a relatively incompressible medium, subjecting them to a high temperature pressure fluid and suddenly releasing the pressure.

2. The step in the preparation of smokeless 15 powder which consists in filling each fiber of a mass of collapsible cellulose fibers with a supporting medium, subjecting them to a high temperature pressure fluid and suddenly releasing the pressure.

3. The step in the preparation of smokeless 20 powder which consists in placing the fibers of a mass of collapsible cellulose fibers in a non-collapsible condition, subjecting them to internal and external pressure and suddenly releasing the 25 external pressure.

4. The step in the preparation of smokeless 30 powder which consists in filling each fiber of a mass of collapsible cellulose fibers with a medium capable of suddenly changing its state and thereby producing a pressure within each fiber and then causing the medium to suddenly change its state whereby the fibers are disrupted.

5. The process of producing cellulose pulp 35 comprising providing cellulose in the form of separate tubular fibers, saturating said fibers with an incompressible liquid so as to fill said fibers with said liquid, then subjecting said fibers to high pressure and temperature, and then suddenly relieving said pressure to cause disruption of said fibers by the vaporization of said liquid.

6. The process of producing cellulose pulp 40 comprising providing cellulose in the form of separate tubular fibers, saturating said fibers with water so as to fill the fibers therewith, then subjecting said fibers to high pressure and temperature, and then suddenly relieving said pressure to cause disruption of said fibers by the vaporization of said water.

6

10

15

20

25

30

35

40

45

50

7. The process of producing cellulose pulp comprising providing cellulose in the form of separate tubular fibers, subjecting said fibers to application of a vacuum for removal of air, then 5 saturating said fibers with an incompressible liquid so as to fill said fibers with said liquid, and

then subjecting said fibers to high pressure and temperature, and then suddenly relieving said pressure to cause disruption of said fibers by vaporization of said liquid.

FREDRICH OLSEN.  
FREDERICK R. SEAVEY.